

April 20, 1937.

C. E. ROZEMA

2,077,714

LUMBER AND METHOD OF MAKING THE SAME

Filed Aug. 28, 1933

*Fig. 1.*



*Fig. 2.*



*Fig. 3.*



*Inventor.*

C. E. Rozema,

*By. Wm G. Frendenreich, Atty.*

## UNITED STATES PATENT OFFICE

2,077,714

LUMBER AND METHOD OF MAKING THE  
SAME

Charles E. Rozema, Grand Rapids, Mich., assignor, by mesne assignments, to Haskelite Manufacturing Corporation, a corporation of New York

Application August 28, 1933, Serial No. 687,122

8 Claims. (Cl. 154—2)

All of the pinaceous or coniferous woods have a tendency to check when exposed to weather. This tendency is very strong in the case of some of these woods, such as fir, cypress, larch, pine, etc., to which group I shall herein apply the name, fir. Fir plywood is a cheap product but its use is limited by its inherent tendency to check. This checking occurs not only in exterior use but also in the case of panels used in interiors. The application of paint somewhat inhibits but does not prevent such checking.

The object of the present invention is to make it possible in a simple manner and at a low cost to prevent visible checking of fir or other wood.

I have discovered that if a piece of fir be faced with strong paper, such as kraft, which will absorb varnish, or other pliable varnish-absorbing cellulosic material, and the facing be then impregnated or partially impregnated with a suitable varnish which is also allowed to extend above the surface of the paper as a continuous film of such varnish, no visible checking develops. Under some conditions the wood may check, but the stresses developed thereby are absorbed by the cellulosic facing layer, so that the varnish film remains intact. Furthermore, the protection afforded to the wood is about the same as though it had thereon several coats of good paint. Therefore, when panels of this kind are used for structural purposes they require no further painting except for color.

The various features of novelty whereby my invention is characterized will hereinafter be pointed out with particularity in the claims; but, for a full understanding of my invention and of its objects and advantages, reference may be had to the following detailed description taken in connection with the accompanying drawing, wherein:

Figure 1 is a view showing the elements to constitute a plywood panel and two facing layers therefor spaced apart from each other and provided with the proper glue coatings, layers or films to produce a three-ply core of wood faced on both sides with paper or other cellulosic material when these elements are glued up in a press; Fig. 2 is an edge view of the panel at the end of the gluing operation; and Fig. 3 is a section, on a greatly enlarged scale, showing a small fragment of the panel after it has been glued, receiving an application of varnish upon one of its faces.

The present invention will be used most widely in connection with plywood panels and, therefore, the detailed description will be confined to this

particular embodiment, although it will, of course, be understood that the invention is not limited to panels or to plywood.

In Fig. 1 of the drawing I have shown three pieces of wood veneer, 1, 2, and 3, adapted to be glued together into a three-ply panel. Layers, films or coatings of glue must be placed between the members 1 and 2 and between the members 2 and 3. The character of the glue in these locations and the manner of applying it may be varied according to the nature of the product desired. In the arrangement shown, the member 2, which may be regarded as the core of the multiple-ply panel, is shown as having been coated on both faces with glue, as indicated at 4 and 5. If the members 1, 2, and 3 are now glued together in a press or otherwise the result will be simply an ordinary three-ply panel which may be regarded as illustrative of multiple-ply panels in general.

In accordance with the present invention another ply is added to form a facing layer. Even though it be not required to guard against checking of both faces of the panel, and since one of the faces could therefore be left in the same condition as heretofore, it is preferable that facing layers be applied to both sides of the panel. Therefore, in assembling the veneers I place underneath the same a facing sheet 6 and lay a similar facing sheet on top of the veneers. The facing sheets must be glued to the wood and this can conveniently be accomplished by coating the upper face of the member 1 with glue, as indicated at 7, and placing a similar glue coating 8 on the under face of the veneer 3. When the five individual pieces appearing in Fig. 1 are pressed together to form a multiple-ply panel, the panel, illustrated in Fig. 2, may be said to consist of five plies instead of three; two of the plies being the facing layers or sheets.

After the panel has been glued it is necessary to treat one or both of the facing layers before the panel is ready for use. This treatment consists in providing coatings in the form of continuous hard protective films so effectively combined with the facing layers that the films cannot be peeled off without destroying the paper or other material of which the facing layers are composed. In order properly to unite the protective film with a facing layer on the panel it is necessary that the facing layer be composed of materials of a kind into which the protective material will readily penetrate while the panel is hot. Then, when a protective material of the proper type is applied to the hot panel, portions

thereof form a film upon the surface of the facing layer and other portions penetrate deeply into the same. Preferably the protective material should permeate the entire facing layer although, if the weaker structure resulting therefrom is not objectionable, the protective material may be allowed to extend only a short distance into the facing layer.

The protective material or materials may be any resinous substance or substances that will exclude moisture, as that is the chief function thereof; the most suitable being synthetic resin varnishes. By varnishes I mean to include, also, lacquers, enamels and paints. Furthermore, although varnishes, lacquers, enamels, etc., ordinarily contain solvents and non-solvents, this is not essential; but dry resinous materials of the proper character and in a fusible condition can successfully be applied to the hot panel. It should therefore be understood that when I refer to a varnish I means any or all of these resinous materials or substances containing them, whether in dry or other form. The resinous component of the "varnish" is preferably of the heat-hardening type.

The facing layers should not be unduly thick, nor should they be too thin. Good results are obtained with strong absorbent paper having a thickness of from three one-thousandths to seven one-thousandths of an inch.

While the glues employed to unite the wood veneers together may be of any usual or suitable kinds, I prefer that the glue lines between the paper and the wood have a high synthetic resin content and that all of the glues be such as to permit the composite panel to be glued up through heat and pressure. It therefore follows that when a panel is removed from the press it is still hot and the absorbent facing layers are in the proper condition readily to absorb varnish deposited upon the same. I prefer to use an aqueous suspension of highly comminuted particles of thermosetting varnish-resin which may be sprayed, brushed or otherwise spread over the exposed surfaces of the facing layers and which dries sufficiently hard for handling while the panel is cooling.

When varnish must be applied to both sides of the panel, this can conveniently be done by running the hot panel through rollers adapted to convey to the surfaces of the hot panel an adequate amount of varnish. However, whether the varnish-resin, with or without solvents or non-solvents, be applied by rollers, by brushing, by spraying, or otherwise, the application of the varnish may be made to one face only where it is not necessary to protect both faces.

The great utility of the present invention will be apparent from the fact that uncoated fir when exposed to weather becomes obviously checked in as short a time as twelve hours, and the further fact that fir provided with three coats of high grade paint shows checks within a very few days under exposure to weather; whereas panels prepared according to my invention have failed to develop cracks or checking through the finished surfaces after exposure to weather for three months. In cases where the paper is saturated and impregnated with resinous materials and is then glued to the fir, the results are not satisfactory because the paper seems to be unable to absorb the stresses set up by the checking of the underlying wood. The reason why this latter method is not satisfactory can readily be understood. When a sheet of paper is thoroughly sat-

urated with a resinous material and is compressed between the plates of a press, the resulting product is a sheet that is hard and brittle and does not possess the character of paper that it did before entering the press; but the sheet is now essentially a film of resin through which cellulosic fibers are distributed. The cellulosic fibers are more or less disintegrated during the pressing operation and thus serve simply as a filler. When stresses are set up in a face veneer of a fir panel to which this impregnated and compressed sheet has been applied, these stresses cannot be distributed throughout any portion of the compressed facing material. The result is that the checks will break through the surfacing layer or, as an alternative, the glue line will be sheared at the junction between the veneer and the surfacing layer. In a panel prepared in accordance with my invention, however, the paper or other cellulosic material retains its original character and acts as a cushion which yields and absorbs the stresses set up in the underlying face veneer.

In Figure 3 of the drawing I have shown the paper in the condition in which it leaves the press as well as in the completed condition. The paper retains its character as a coherent sheet as represented by the right-hand half of the member 6 in Fig. 3; this sheet being simply united to the adjacent face veneer 1 by a glue line 10. The varnish-resin material is shown as being supplied in the form of a spray C, in sufficient quantity to cause the paper to be permeated down to the glue line 10, as indicated at 11, and leave a thin continuous superficial protective film 12 upon the paper. Since the varnish-resin extends down to the glue line, the paper is strengthened in the vicinity of the glue line while retaining the elastic properties characteristic of the paper fiber.

While I have illustrated and described with particularity the best form of my invention and the best mode of carrying it out, I do not desire to be limited to the details thus illustrated and described; but intend to cover all methods and materials coming within the definitions of my invention constituting the appended claims.

I claim:

1. The method of producing a product that will not check of wood having a tendency to do so, which comprises gluing to a face of the wood by the hot process pliable cellulosic material that will absorb varnish when such material is hot, and while the said material is still in a heated condition, applying varnish to said material to cause portions thereof to penetrate into said material and the remainder to form a continuous film overlying the cellulosic material.

2. The method of producing a product that will not check of wood having a tendency to do so, which comprises gluing to a face of the wood pliable cellulosic material that will absorb varnish, and applying varnish compatible with the glue to said material while the latter is in a heated condition.

3. The method of producing a material that will not check of wood having a tendency to do so, which comprises gluing to a face of the wood paper that will absorb varnish and applying sufficient varnish compatible with the glue to the paper while the paper is in a heated condition to cause portions to penetrate into the paper in the vicinity of the glue line and the remainder to form a continuous film overlying the paper.

4. The method of producing a product that will not check of wood having a tendency to do

so, which comprises gluing to a face of the wood by means of glue having a high resin content paper that will absorb varnish and, while the paper is in a heated condition, applying varnish resin to the paper.

5. The method of producing a plywood panel that will not check of wood having a tendency to do so, which comprises gluing up by a hot process a plywood panel and facing layers therefor composed of pliable cellulosic material and, while the panel is still hot, applying varnish-resin to one or both of the facing layers.

6. The method of producing a plywood panel that will not check of wood having a tendency to do so, which comprises gluing up by a hot process a wood panel and a facing layer therefor composed of cellulosic material between which and the wood there is a glue line having a high resin content and, while the panel is still hot, applying 15 varnish-resin to the facing layer.

20 7. The method of producing a plywood panel

that will not check of wood that has a tendency to do so, which comprises gluing up by a hot process a wood panel and facing layers of strong paper that will absorb varnish and between which facing layers and the body of the panel are glue 5 lines having a high resin content and, while the panel is still hot, applying varnish-resin to one or both facing layers.

8. The method of producing a plywood panel that will not check of wood that has a tendency to do so, which comprises gluing up by a hot process a wood panel and facing layers of strong paper that will absorb varnish and between which facing layers and the body of the panel are glue 10 lines having a high resin content and, while the panel is still hot, applying to the facing layers an aqueous suspension of varnish-resin in highly 15 comminuted form.

CHARLES E. ROZEMA. 20